

Patented Nov. 27, 1934

1,982,277

# UNITED STATES PATENT OFFICE

1,982,277

## MOTOR FUEL AND METHOD OF PREPARING SAME

Carl Winning, Elizabeth, N. J., assignor, by mesne  
assignments, to Gasoline Antioxidant Company,  
Wilmington, Del., a corporation of Delaware

No Drawing. Application April 24, 1931,  
Serial No. 532,707

6 Claims. (Cl. 44—9)

The present invention relates to an improved naphtha, more specifically to an improved gasoline line which has been made stable against gum formation by the addition of small amounts of 5 aromatic nitroso compounds. The invention will be fully understood from the following description:

It has long been well known in the petroleum industry that low boiling hydrocarbon oils such 10 as gasoline and naphtha, especially cracked gasoline and naphtha, often contain gum or gum forming constituents in harmful quantity. In the following description, the oil to be treated will be referred to as low boiling hydrocarbon oil or 15 naphtha.

Naphthas containing large quantities of gum, or constituents tending to form gum during storage, are objectionable for many purposes, such as for motor fuels, light solvents, etc. Recently 20 a careful study of gum formation has been made by petroleum chemists, and several organic compounds have been found which, when added in small quantities to low boiling hydrocarbon oil, will retard or inhibit gum formation for periods 25 of time varying with the nature of the compound, the oil, and other conditions.

The usual test for such gum forming constituents is known as the copper dish method and is described on page 96 of the United States Bureau 30 of Mines Technical Paper No. 323 D, revised October 21, 1927. The result of this test is expressed in milligrams of gum left in the dish on evaporation of 100 cc. of naphtha.

Another testing method consists of adding 35 oxygen under pressure to the sample of the low boiling hydrocarbon oil to be tested in a closed vessel, and then keeping the oil at elevated temperature of say 100° C. under a pressure of oxygen of say 100 lbs. per square inch. For a certain 40 time the pressure remains practically constant, then it begins to drop suddenly. This drop is observed on a pressure gage. The period of time during which no pressure drop is observed is called the induction period. The 45 longer this induction period, the better is the particular oil tested, and the less likely it is to form gum during storage.

An approximate quantitative relation for the 50 gum inhibiting power of a certain inhibitor may be expressed by the following equation:

$$I.P. = \frac{S-B}{B} \times \frac{1}{C}$$

where I. P.=inhibiting power

S=induction period of solution

B=induction period of blank or solvent

C=concentration of the inhibitor in %

by weight.

The test just described is quicker and more 60 reliable, and gives more readily reproducible

data, than the copper dish method. The I. P. number of an inhibitor will accordingly be used herein as a measure of its value. It will be understood, however, that the inhibitors of the present invention may be rated according to the copper dish method, or other suitable method, and will show a corresponding value. Moreover, these inhibitors are effective in actual storage tests, that is, when added to naphtha stored in the tanks of refineries or distributors. The oxidation test described herein gives an accelerated indication of the performance to be expected during storage.

I have discovered that aromatic nitroso compounds and such mixed derivatives as nitroso phenols and nitroso amines are good gum inhibitors. When mixed derivatives such as nitroso amines or nitroso phenols are used it is preferable to have the amino or hydroxyl in the para or ortho position to the nitroso group. Many suitable nitroso derivatives exist such as dinitroso resorcinol, nitroso naphthol, para-nitroso dimethyl aniline, alpha-nitroso beta-naphthol, beta-nitroso alpha-naphthol, etc. Some of the aromatic derivatives containing a nitroso group may also impart color to the naphtha, and dyes containing the nitroso group may also be used.

Compounds of the class described above will give an efficient protection against gum formation in a gasoline during ordinary storage for a long period of time when added in amounts of from 0.0005 to 0.1% by weight of the oil. The necessary amounts are best determined empirically. Compounds of the type described are in general sufficiently oil soluble and may be readily distributed uniformly throughout even large bodies of oil by simple mixing. If desirable they may be dissolved in benzene or other suitable solvent from which they will not be readily precipitated by access of moisture. The solution so prepared may be mixed with the oil.

The following example will illustrate the improvement obtained in gum inhibitors by the introduction of a nitroso group. Dimethyl aniline is a comparatively poor gum inhibitor which has an I. P. number of 35. Para-nitroso dimethyl aniline, on the other hand, is a good gum inhibitor having an I. P. number of 250.

My invention is not to be limited by any theory nor by the examples given as illustrations but only by the following claims in which it is my intention to claim all novelty inherent in my invention.

I claim:

1. A motor fuel comprising cracked gasoline normally tending to deteriorate and form gum, and containing a small quantity of a gum inhibiting agent selected from the group consisting of dinitroso polyhydroxy benzenes, nitroso naphthols wherein the nitroso and hydroxyl

65

70

75

80

85

90

95

100

105

110

115

120

groups are on adjacent carbon atoms, and a

nitroso aniline.

2. The method of preserving cracked hydro-carbon distillates which deteriorate and develop 5 gum on storage, by incorporating therein a small proportion of an organic reducing agent selected from the group consisting of dinitroso polyhydroxy benzenes, nitroso naphthols wherein the nitroso and hydroxyl groups are on adjacent 10 carbon atoms, and a nitroso aniline.

3. A motor fuel comprising cracked gasoline which normally tends to deteriorate and form 15 gum upon storage and containing a small quantity of a nitroso aniline in quantity sufficient to retard such deterioration and gum formation.

4. A motor fuel comprising cracked gasoline

normally tending to deteriorate and form gum upon storage and containing a small quantity of a nitroso naphthol selected from the group consisting of alpha-nitroso-beta naphthol and beta-nitroso-alpha naphthol.

80

5. A cracked naphtha normally tending to form gum during storage and stabilized against gum formation by the addition of 0.0005 to 0.1 per cent by weight of para-nitroso dimethyl aniline.

85

6. A cracked naphtha normally tending to form gum and stabilized against gum formation by the addition of 0.0005 to 0.1% by weight of di-nitroso-resorcinol.

CARL WINNING. 90

90

20 95

25 100

30 105

35 110

40 115

45 120

50 125

55 130

60 135

65 140

70 145

75 150